

Dec. 11, 1928.

1,695,038

O. E. BUCKLEY

MAGNETIC ALLOY

Filed March 6, 1925

Fig. 1



Fig. 2



Inventor:  
Oliver E. Buckley

by Edward A. Adam, Atty.

## UNITED STATES PATENT OFFICE.

OLIVER E. BUCKLEY, OF MAPLEWOOD, NEW JERSEY, ASSIGNOR, BY MESNE ASSIGNMENTS, TO WESTERN ELECTRIC COMPANY, INCORPORATED, A CORPORATION OF NEW YORK.

## MAGNETIC ALLOY.

Application filed March 6, 1925. Serial No. 13,501.

This invention relates to the production and use of a new material or substance having certain desirable magnetic and electrical qualities the chief one of which is high permeability, especially at low magnetizing forces, which is relatively independent of mechanical stresses applied to the material. This material is an alloy containing nickel and iron and properly heat treated to give it the desired high permeability.

In the Patent No. 1,586,884, issued June 1, 1926, to G. W. Elmen, there is disclosed a magnetic alloy consisting in its preferred proportions of 78½% nickel and 21½% iron which, when given a specified heat treatment, has remarkably high permeability at low magnetizing forces. It is also there disclosed that the alloy should be guarded against undue stresses and strains after it has been heat treated to develop high permeability; as the permeability is somewhat affected by such stresses and strains. Other alloys of nickel and iron in which the nickel content is somewhat less are even more sensitive to strain.

In the present application, which is a continuation in part of my application Serial No. 697,584, filed March 7, 1924, the chief object of the invention is the production of an alloy having one or more of the desirable characteristics of the alloy described in the above mentioned Elmen application but one which is much less sensitive to strain. Other objects will appear from the following description.

In the accompanying drawings, Fig. 1 is a set of curves showing the relationship between tension and permeability of various nickel-iron alloys, and Fig. 2 shows a section of a submarine cable in which the improved material is utilized for inductive loading.

When a study was made of the effects of tension upon nickel iron alloys having from 65% to 90% nickel and the rest iron and all being given the same treatment to secure as great uniformity and freedom from internal strain as possible, it was discovered that if the nickel content was less than 80% or thereabout, the permeability increased with tension while if the nickel constituted above 80% or thereabout, the permeability decreased with tension, but in the composition containing approximately 80% of nickel, the permeability was very nearly independent of the tension applied. Later investigation

showed that the composition of the alloy in which the permeability is most nearly independent of tension varies somewhat with the heat treatment, as explained in the following specification. The accompanying drawing is a series of curves showing the relation between permeability at a magnetizing force of .01 gauss and applied tension for various compositions of nickel and iron.

In the above mentioned patent to G. W. Elmen and in the Patent No. 1,586,874, issued June 1, 1926, to O. E. Buckley, there are described many uses for such nickel-iron alloys, one of the principal uses being as a loading material for increasing the inductance of signaling conductors and especially transoceanic submarine cables. The magnetizing forces set up by the signaling current in such a cable ordinarily varies from around two tenths c. g. s. unit (gauss) at the sending end to about .001 gauss near the middle and to exceedingly small values at the receiving end. As fully set forth in the Buckley patent, the properties of these alloys in their preferred proportions peculiarly adapt them for use as loading material for long submarine cables and it was in connection with such use that the research leading to this invention was undertaken. The loading is preferably placed upon the cable conductor in the form of a layer of helically wrapped tape or wire. One manner of doing this is disclosed in Patent No. 1,586,887, issued June 1, 1926, to G. W. Elmen. The loaded conductor is passed through an electric furnace which is maintained at a temperature of about 900° C., and, as it emerges from the furnace, is cooled at the proper rate to give the material high permeability at low magnetizing forces of the order encountered in submarine signaling. It would be of advantage to heat treat the tape in a manner to secure high permeability before applying it to the conductor were it not for the fact that wrapping the tape around the conductor introduces strains in it which greatly lower the permeability.

The inductance of the loaded conductor, moreover, was found to be varied by deep water pressure unless special means was employed to equalize this pressure in a manner to relieve the conductor from strain. This means is described and claimed in Patent No. 1,586,875, issued June 1, 1926, to O. E. Buckley.

With the idea in mind that by varying the composition of the nickel iron alloy a material might be found which would possess as high permeability as that of the alloy here-  
 5 tofore used and not be subject to the objections to that alloy resulting from its sensitiveness to strain, measurements were made on wires so arranged that their permeabilities could be measured while the material  
 10 was under tension of any desired amount. The type of strain used was that resulting from simple tension on the material. This was chosen for the sake of simplicity in experimental procedure and interpretation of  
 15 results. The wires tested constituted a grad-  
 ed series of nickel iron alloys extending from 65% nickel to 90% nickel. The invention however is not limited to strains introduced by tensions.  
 20 The heat treatment given to the wires was as follows: The samples were placed in a quartz container which was then evacuated and inserted in a furnace which was main-  
 25 tained at a temperature of approximately 960° C. After being in the furnace about ten minutes the container was removed and allowed to cool slowly to room temperature before being opened. No attempt was made to obtain the highest possible permeability.  
 30 These experiments disclosed the existence of a narrow range in the neighborhood of 80% to 83% nickel in which the change of  
 35 permeability with tension is relatively small and on one side of which permeability in-  
 creases with tension while on the other side it decreases. The results of the tests are  
 40 shown in the curves of the drawing. Al-  
 though the curves show a maximum tension of 2000 pounds per square inch, the tests were  
 45 actually conducted up to tensions of about 10,000 pounds per square inch without caus-  
 ing any marked variation in the curve rep-  
 resenting the behavior of 80% nickel and  
 50 20% iron. Data were obtained also on an  
 alloy comprising 81% nickel and 19% iron  
 for field strengths up to six gauss and though  
 the permeability changes within this range  
 55 in a manner similar to that of the preferred  
 composition of the above-mentioned Patent  
 60 No. 1,586,884 to G. W. Elmen, and shown for  
 example in a paper by Arnold and Elmen en-  
 titled "Permalloy," Journal of Franklin In-  
 65 stitute, May, 1923, no marked variations  
 were produced in the shapes of the curves giv-  
 ing the relation of permeability to tension  
 at a fixed field strength. The permeability  
 70 of the 80% nickel composition was around  
 4,000 at  $H = .01$  gauss as shown in the draw-  
 ing and the initial permeability of this ma-  
 75 terial was around 3800. It is interesting also  
 to note that although the effects of tension  
 on the permeability of pure iron and pure  
 nickel are comparatively less than for these  
 80 alloys, the direction of the tension effect in  
 85 alloys having more than 80% nickel is the

same as that in pure nickel and the behavior of the alloys of more than 20% iron is like that of iron in low magnetic fields.

Further experiments were conducted to de-  
 70 termine what effect if any would result from  
 the addition of other ingredients in small  
 amounts which might either be present as im-  
 purities, or which might be purposely added  
 to alter characteristics of the material, such  
 75 for example, as the addition of small amounts  
 of chromium to increase the resistivity of the  
 material or the addition of copper to alter  
 its mechanical properties. The results of  
 these tests indicate that the insensitivity of  
 80 the material to strain is not materially affect-  
 ed by the addition of other ingredients in  
 small percentages so long as the proportion  
 of nickel in the alloy remains approximately  
 85 80% of the combined nickel iron content.

The exact ratio of nickel to iron however,  
 86 to obtain this result depends somewhat upon  
 the strength of field to which the material is  
 to be subjected but will probably lie within  
 the limits of 80% to 83% nickel and 20% to  
 90 17% iron. Thus, for example, with an alloy  
 of 81% nickel and 19% iron, the sign of the  
 95 effect of tension upon magnetization changes  
 several times during the process of magneti-  
 cally saturating the material, although the  
 degree of sensitivity to strain is very slight  
 100 over the entire range.

The experiments in stronger fields showed  
 105 also that at about that composition which  
 possesses the least variation with tension of  
 permeability in low fields, the coercive force  
 and the area of the hysteresis loop were also  
 110 least affected by tension. For alloys contain-  
 ing less than 80% of nickel, the effect of ten-  
 sion is to reduce the coercive force and the  
 hysteresis loss per cycle. In the case of alloys  
 115 containing more than 80% of nickel, the ef-  
 fect of tension is to increase the coercive force  
 and the hysteresis loss per cycle. It is under-  
 120 stood in both cases that coercive force and  
 the hysteresis losses compared are those ob-  
 125 tained from measurements carried to the  
 same maximum induction.

The resistivity of the alloy comprising 80%  
 130 nickel and 20% iron was found to be about  
 $16 \times 10^{-6}$  ohms per cm. The other alloys  
 tested showed a change in resistivity in the  
 same direction as the change in permeability  
 when tensions were applied. The resistivity  
 135 of the 80% nickel composition remained sub-  
 stantially constant, a property which, while  
 not so important in general as that of stabili-  
 zation of permeability, since the resistivity  
 is not so sensitive to strain, is nevertheless  
 140 important.

Fig. 2 shows a portion of a submarine cable  
 145 inductively loaded with an alloy such as that  
 just described. Such a cable is described at  
 length in the Patent No. 1,586,874 to O. E.  
 Buckley, referred to above. In this figure  
 150 a central copper conductor 1 is surrounded

by copper strands 2 making a composite stranded conductor. Tape composed of the improved alloy is wound helically about the conductor 1 forming a layer 3 of inductive loading. This in turn is surrounded by gutta percha insulation 4 and the usual armoring and protective covering 5.

The new alloy is particularly well adapted for this use where very high permeability is desired as it is found that the highest permeability is obtained in practice if the alloy is of the composition which is relatively insensitive to strain. By testing various compositions of nickel-iron alloys by themselves, apart from the conductor, it has been found that the highest initial permeability is obtained by special heat treatment of a composition of 78½% nickel and 21½% iron. However, by testing tapes of the various compositions applied to a copper conductor and then heat treated, it has been found that the highest inductance for small currents and therefore the highest actual permeability is obtained with a composition in which the nickel content is 80% to 81% of the nickel-iron content. The reason for the latter composition giving better results in the case of the loaded conductor is thought to be its smaller sensitiveness to strain. In the cooling stage of the heat treatment, there is a tendency for the nickel iron loading material to adhere to the copper conductor with the consequent introduction of mechanical strain. This fact is apt to be particularly pronounced if the loading material is applied tightly to the conductor. The strain introduced by adhesion impairs the desired characteristics of the alloy of 78½% nickel and 21½% iron much more than alloys of 80% to 81% nickel and 20% to 19% iron which, as has been pointed out above are relatively insensitive to strain. The result is that a higher final inductance is secured with the insensitive alloy. Alloys of the insensitive range are also particularly well adapted for use on submarine cables since they are not affected by the high pressures encountered in deep water to the same degree as are other alloys, for example, the 78½% nickel and 21½% iron.

What is claimed is:

1. A nickel iron alloy comprising nickel and iron, the nickel being between 80% and 83% of the total iron-nickel content, and having higher permeability than iron at magnetizing forces less than a few tenths of a c. g. s. unit.

2. A magnetic alloy comprising materials having an electric or magnetic property which varies in one direction in one of said materials and in the opposite direction in another of said materials under varying applied mechanical forces over a certain range, said alloy containing said materials in the proper proportions so that the effects of such me-

chanical forces are balanced, whereby the property in question of the alloy may be substantially independent of applied mechanical forces over the said range.

3. A magnetic composition mainly comprising nickel and iron with nickel predominating and which has been heat treated to have a permeability greater than that of iron at magnetizing forces of a few tenths of a gauss and substantially independent of applied mechanical forces up to the point where the elastic limit is reached.

4. A magnetic alloy which has a permeability greater than that of iron at magnetizing forces of a few tenths of a gauss comprising from about 80% to 83% nickel and the remaining portion chiefly iron, said permeability being more nearly independent of applied mechanical forces than when the nickel component is either increased or reduced.

5. A magnetic alloy which has a higher permeability than iron at magnetizing forces of a few tenths of a gauss or less comprising from about 80% to 83% nickel and the rest iron, said permeability being substantially independent of tension over a wide range.

6. A magnetic composition which has a higher permeability than iron at magnetizing forces of a few tenths of a gauss or less and high permeability at forces of the order of 1. gauss comprising from about 80% to 83% nickel and the rest iron, said permeability being substantially independent of tensions from zero to at least 5000 pounds per square inch.

7. An alloy, the greater part of which is nickel and the rest chiefly iron and which has been heat treated to have a permeability greater than that of iron at a magnetizing force of a few tenths of a gauss and a resistivity which is substantially independent of applied mechanical forces over a wide range.

8. An alloy, the greater part of which is nickel and the rest chiefly iron which has been heat treated to have a permeability greater than that of iron at magnetizing forces of a few tenths of a gauss and so that the permeability and resistivity are nearly independent of applied mechanical forces over a wide range.

9. The combination with an electric conductor of magnetic material associated therewith comprising an alloy containing principally nickel and iron, the amount of nickel present constituting from 80% to 83% of the total nickel iron contents.

10. A signaling conductor comprising a central conducting member having magnetic loading material associated therewith, said material consisting of an alloy containing principally nickel and iron in which the amount of nickel present is from 80% to 83% of the total nickel iron content.

11. A method of preparing a magnetic al-

loy which has the characteristic of constant permeability independent of mechanical strain, which consists in combining in alloy form a magnetic material in which the permeability normally increases in strain, with a magnetic material in which the permeability decreases in strain in such proportions as to cause the strain permeability characteristics of one element to balance the strain permeability characteristics of the other element.

12. A continuously loaded signaling conductor comprising a conducting member

having associated therewith a magnetic loading material which consists mainly of nickel and iron, with nickel predominating and which has been heat treated before its association with said member to have a permeability which is higher than that of iron and which is substantially unimpaired by the process of said association.

In witness whereof, I hereunto subscribe my name this 5th day of March, A. D., 1925.

OLIVER E. BUCKLEY.

15

20